

5-121

# UNITED STATES PATENT OFFICE.

MARCELLO VON PIRANI, OF WILMERSDORF, NEAR BERLIN, GERMANY, ASSIGNOR  
TO GENERAL ELECTRIC COMPANY, A CORPORATION OF NEW YORK.

## METHOD OF WORKING REFRACATORY METALS

1,089,786.

No Drawing.

Specification of Letters Patent. Patented Mar. 10, 1914.

Application filed November 23, 1912. Serial No. 733,076.

To all whom it may concern:

Be it known that I, MARCELLO VON PIRANI, a citizen of the Italian Kingdom, residing at Wilmersdorf, near Berlin, Germany, have 5 invented certain new and useful Improvements in Methods of Working Refractory Metals, of which the following is a specification.

In the working of refractory metals such 10 as tungsten, as by rolling, it is observed that the material under treatment becomes cracked after a certain amount of rolling, the cracks formed being principally longitudinal. The formation of cracks may be to 15 such an extent that pieces come entirely away from the material being rolled. In consequence of this phenomenon it becomes necessary to do the rolling with extreme care which increases the length of time consumed in the operation and also the cost of 20 the work. If great care is not exercised a large percentage of waste results since the cracked pieces cannot be further rolled but must be remelted or otherwise utilized. This 25 difficulty is remedied by the following method: As soon as cracks or fractures appear in the material being rolled the operation is interrupted and the material heated to such a point that the cracks sinter or 30 melt together; thereby not only does the surface of the piece being rolled become smooth, but if the temperature is carried sufficiently high the cracks may be completely sintered together so that the metal 35 again presents a uniform character throughout. If the piece of metal so treated is again brought into the rolls it behaves like new, unrolled material.

The heating of the metal will give the best 40 results if it is not carried on throughout the entire mass of the material rolled, but only at the place where the crack occurred and where it is desired that the metal be resintered, the character of the remaining parts 45 of the metal will therefore be little changed. It is necessary therefore only to heat the edges and surfaces of the cracks whereby they will be reunited.

One method of carrying out this invention 50 is as follows: The piece to be rolled is heated

by the electric current. It serves as one electrode and another electrode is moved over the place to be heated. By this means the effect of the heat can be closely confined and its intensity finely regulated. The heating 55 may be effected in a hydrogen atmosphere in order to avoid oxidization.

The phenomenon of cracking is particularly noticeable when the rolling process lasts a long time and the material is thereby 60 considerably cooled, but in rolling metals in which the cooling is not a substantial feature—the rolling being effected at a low temperature—such cracks may form but to a less extent.

What I claim as new and desire to secure by Letters Patent of the United States is:—

1. The process of reclaiming refractory metal which has become cracked during rolling which consists in locally heating the 70 metal to a temperature sufficient to cause the crack to be completely and automatically eliminated merely by heating until said cracked portion becomes homogeneous, and re-rolling said metal.

2. The process of reclaiming refractory metal which has become cracked during rolling which consists in electrically locally heating the same in an inert atmosphere to a point sufficient to cause the cracked portions 80 to automatically reunite into a homogeneous body of metal, and re-rolling said metal.

3. The process of reclaiming refractory metal which has become fractured during rolling which consists in locally heating the 85 metal by electricity in an inert environment by connecting said metal to one pole of a source of current, and moving an electrode connected to the other pole of said source over said metal adjacent the fracture, and 90 thereby raising said metal to a sufficient temperature to cause the imperfect portions to sinter together, and re-rolling said metal.

In witness whereof, I have hereunto set my hand this 5th day of November 1912.

MARCELLO VON PIRANI.

Witnesses:

HENRY HASPER,  
WOLDEMAR HAUPT.

Copies of this patent may be obtained for five cents each, by addressing the "Commissioner of Patents.  
Washington, D. C."